

# UNITED STATES PATENT OFFICE.

ANTENORE FUSAI, OF BIELLA, ITALY, ASSIGNOR TO ALFREDO BALADA, OF SAME PLACE.

## MANUFACTURE OF FELT.

SPECIFICATION forming part of Letters Patent No. 680,522, dated August 13, 1901.

Application filed February 1, 1900. Serial No. 3,633. (No specimens.)

To all whom it may concern:

Be it known that I, ANTENORE FUSAI, a subject of the King of Italy, residing at Biella, in the Kingdom of Italy, have invented certain new and useful Improvements in the Manufacture of Felt; and I do hereby declare that the following is a full, clear, and exact description of the same.

This invention aims to provide a new treatment for vegetable fibers to render them capable of use in the manufacture of felt.

It aims to provide especially new materials for the manufacture of felt and a new process of manufacturing felt therefrom.

15 It aims to provide also a felt composed of a new material.

The new materials referred to are the vegetable wool or silk fibers known in the trade as "Kapok" and "Ceiba." These fibers 20 have a roughness not found in cotton and have some analogy to wool, though somewhat finer, brighter, and softer. The fiber is pierced by a channel of about one-tenth of its diameter. While the fiber of cotton is some-

25 what flat, that of kapok and ceiba is quite round and rough on its surface, whence the possibility of using it in the manufacture of felt. The central channel is empty, as in cotton, while that of wool is filled with medul-

30 lary matter. Though similar to wool on its surface, the new fiber is somewhat smaller. Kapok is the fiber which forms the involucre of the seed of the *Eriodendron anfractuosum*, a tree growing in tropical countries. Ceiba

35 is obtained from the ceiba tree, which is common in Honduras. According to the process of this invention such fibers are rendered capable of felting by submitting them after a thorough cleansing to chemical processes ex-

40 erting, oxidating, disintegrating, and roughening action upon the outer portion thereof, so as to render them capable of felting. This action is effected by means of baths, the first of which contains mercury in solution.

45 The second bath contains chromic acid and is made from substances capable of developing such acid—such, for example, as bichromate of potash, from which chromic acid can be developed by sulfuric acid. To this

50 bath may be added other substances possessing properties such as fit them to coöperate

to improve the felting qualities of the fiber—such, for instance, as gallic acid, nitric acid, and hydrochloric acid and their compounds or derivatives. In conjunction with these 55 acids there may be employed tannin or *enocianine*, (the coloring-matter of wine,) or sulfate of copper, or of iron, or their components or derivatives. The proportions of the said materials vary in the preparation of the 60 baths, according to the fineness and quality of the felt to be made. If, for example, a good hat-felt is wanted, the vegetable fibers must be submitted, after cleaning, to a first bath composed, approximately, as follows: 65 One thousand parts, by weight, of nitric acid, two hundred and fifty of mercury, and three thousand of water. This bath imparts a yellow color, usually called "yellow secrete," to the fiber on account of the oxidation of the 70 nitrate of mercury dissolved in the bath and its adherence to the fiber in the form of an insoluble precipitate. When a large proportion of water is employed, the yellow coloration is pale or pallid and is called "pallid secrete." 75 This solution is employed in the proportion of from two to three parts, by weight, to one hundred parts, by weight, of water to each two parts, by weight, of the vegetable fibers, the bath being at a temperature of about 40° centigrade. The said fibers are first saturated with water. The vegetable fibers are allowed to remain in this bath for a time, usually about ten to fifteen minutes, and they are 80 then removed from the bath and placed and allowed to remain in another vessel for about twenty-five hours to dry them and then they are submitted to the action of a second bath composed of bichromate of potash, two to six per cent., by weight, of the weight of fiber 85 treated; tannic acid, one to two per cent.; acetic acid, one to two per cent.; water, twenty-five times the weight of fiber treated, and acid coloring-matters of the desired color and in a quantity corresponding to the degree of 90 coloring desired. The vegetable fibers are plunged into said second bath at a temperature of about 40° centigrade, and then the temperature is raised to about 90° centigrade. After they have remained from ten 95 to fifteen minutes at this temperature they are removed to another vessel, where they are 100

allowed to stand alone for about twenty-four hours and, lastly, dried and blown by the ordinary processes. A further action may be exerted upon the fibers so prepared by means 5 of sulfuric acid during the fulling. The ordinary doses of sulfuric acid must be increased not less than one-third, and it will be well to add in the fulling-machine one per cent. of bichromate of potash, tincture 10 of *enocianina* or other oxidizing disintegrating and roughening agents, and coloring matters which will vary in quality and proportions in accordance with the requirements of practice. The preparation of the baths depends also upon the quality and strength of 15 the chemical preparation (pallid or yellow secrete) taken up by the fibers.

It may be said, as a rule, in the treatment of mixtures of animal and vegetable fibers 20 that starting from the hereinbefore-stated formulas as adapted to the manufacture of a felt for a hat the doses of these formulas must be increased in proportion with the quantity of vegetable fiber employed. 25 For the manufacture of felt for clothes, caps in general, carpets, shoes, &c., the above formulas are susceptible of reduction if, as animal material, wool is employed, the wool having re-entering properties much greater 30 than the hair of the hare and the rabbit and being capable, with a small help of disintegrating or roughening agents, of bringing the vegetable materials to the desired point of felting. 35 In the manufacture of coarse felts—as felts for paper-mills, horse-clothes, beds, &c.—where very coarse animal material is used, which is little adapted by itself to cause the vegetable material to form into felt, the doses 40 of the roughening materials must be increased and for every special case a special mixture of them be combined, so as to obtain the desired result.

To improve the felting of the vegetable 45 hair and its combination with the animal hair, it may be useful to mix with the vegetable fibers (before preparing them) the detritus of animal materials—for instance, the remainders and the offscourings of hats, residues 50 from the manufacture of felt, clippings, &c. Said offscourings are first passed into a strongly-acid bath (sulfuric and nitric acids) to break down the fibers too large and un-felted. Afterward they are put very quickly

into an alkaline bath and washed in abundant 55 pure water. The said residues when so treated are ready to be employed and when dried are employed by mixing them in the proportions of from five to forty and even fifty per cent. with the vegetable fibers. 60

The vegetable fibers properly prepared, as hereinbefore described, either alone or mixed with residues of animal fibers, are felted with the animal fibers by intercalating strata of the same among strata of vegetable fibers, 65 leaving on each outer side of the finished felt a stratum of animal felt, so that the felt looks from the outside exactly like a felt fully made of animal fiber.

Instead of the intercalation of the strata a 70 direct mixture of the vegetable and animal fibers might be made; but the intercalation as described is preferred.

Usually in manufacturing felt for hats a 75 stratum of vegetable fibers is placed between two of animal fibers. Also certain qualities of felts can be made simply of vegetable fibers prepared as hereinbefore described, either alone or mixed with residues of animal fibers. 80

No further particulars as to the finishing of the felt are added here, as it can be effected by any of the known processes.

Having thus described my invention, what I claim as new therein, and desire to secure 85 by Letters Patent, is—

1. The process of rendering vegetable fiber such as kapok or ceiba capable of felting, which consists in treating the fiber first with a bath containing mercury, and then with a 90 bath of substances capable of developing chromic acid, and in then drying the same.

2. The process of rendering vegetable fiber such as kapok or ceiba capable of felting, which consists in treating the fiber first with a 95 bath containing mercury, and then with a bath of substances capable of developing chromic acid to which have been added disintegrating and roughening agents substantially as specified, and in then drying the 100 same.

In witness whereof I have hereunto signed my name in the presence of two subscribing witnesses.

ANTENORE FUSAI.

Witnesses:

YAIRO CAPUNI,  
ENRICOE MARAVA.